# EUROPEAN PATENT SPECIFICATION

(11) **EP 2 269 208 B1**
(45) Date of publication and mention of the grant of the patent: **20.03.2013**
(21) Application number: 09739151.0
(22) Date of filing: 28.04.2009
(51) Int. Cl.: H01J 9/00

(54) **APPARATUS AND METHODS FOR USE OF REFRACTORY ABHESIVES IN PROTECTION OF METALLIC FOILS AND LEADS**
VORRICHTUNG UND VERFAHREN ZUR VERWENDUNG FEUERFESTER HAFTUNTERDRÜCKER ZUM SCHUTZ VON METALLFOLIEN UND -BLECHEN
APPAREIL ET PROCÉDÉS POUR UNE UTILISATION D'AGENTS ANTI-ADHÉRENTS RÉFRACTAIRES DANS LA PROTECTION DE FEUILLES ET DE FILS MÉTALLIQUES

(30) Priority: 28.04.2008 US 71417
(43) Date of publication of application: 05.01.2011
(73) Proprietor: Advanced Lighting Technologies, Inc., Solon, OH 44139 (US)
(72) Inventor: EMILSSON, Tryggvi, Champaign, IL 61820 (US); VOGGENAUER, Nikolaus, Fithian, IL 61844 (US)
(74) Representative: Liesegang, Eva
(86) International application number: PCT/US2009/002573
(87) International publication number: WO 2009/134348

(56) References cited:
- GB-A- 671 178
- GB-A- 1 521 129
- US-A- 707 723
- US-A- 3 693 241
- US-A- 5 340 448
- US-A- 5 536 991
- US-A- 5 754 005

## Description

### RELATED APPLICATIONS

The instant application is a continuation-in-part application and claims the filing-date benefit of co-pending U.S. Patent Application No. 11/545,469, filed October 11, 2006 which is a divisional application of and claims priority to U.S. Patent Application No. 10/702,558, filed November 7, 2003, now U.S. Patent No. 7,153,179, which claims the filing-date benefit of U.S Provisional Patent Application No. 60/424,338 filed November 7, 2002.

The instant application also claims the filing-date benefit of U.S. Provisional Patent Application No. 61/071,417 filed April 28, 2008. .

### BACKGROUND

The present subject matter generally relates to electrical lead assemblies in devices such as electric lamps for providing an electrical path through a hermetic press, pinch, or shrink seal formed in a vitreous material such as fused silica or hard glass.

In certain devices, it is often necessary to provide an electrically-conducting path through a pinch or shrink seal formed in a vitreous material. For example, in devices such as electric lamps, e.g., halogen incandescent filament bulbs and high intensity discharge ("HID") arc tubes, a light emitting chamber is formed from a vitreous material having one or more pinch seals that hermetically seal the chamber. In such lamps, one or more electrically-conducting paths from the interior of the chamber to the exterior of the chamber are typically formed by positioning an electrical assembly in one or more of the portions of the tube, and "pinching" the tube to form a hermetic seal around a portion of the assembly. The electrical lead assembly typically includes a metallic foil having electrically conducting leads mechanically secured to the foil and extending from each end thereof. The assembly is positioned so that the foil forms the electrically conducting path through a portion of the vitreous material that has been pinched or shrunk together to form a hermetic seal.

Although any suitable material may be used, typically, the foil in such electrical lead assemblies is formed from molybdenum because of its stability at high temperatures, relatively low thermal expansion coefficient, good ductility, and sufficient electrical conductivity. However, molybdenum oxidizes rapidly when exposed to oxygen at temperatures greater than about 350°C. Since the foils in electrical lead assemblies in electric lamps are often exposed to temperatures greater than about 350°C, the metallic foil may be highly susceptible to oxidation resulting in a breach of the electrical path or the gas-tight integrity of the hermetic seal resulting in lamp failure. Typically, a molybdenum foil exposed to a reactive atmosphere will not oxidize appreciably below about 350°C. At temperatures greater than about 350°C, the rate of the reaction between the oxygen in the surrounding atmosphere and the molybdenum foil greatly increases resulting in corrosion of the foil and a substantial reduction in the useful life of the lamp. Areas particularly susceptible to such oxidation include the spot weld connecting the outer lead to the foil and the area on the foil adjacent the outer lead.

Figure 1a is a schematic representation of a conventional arc tube for a high intensity discharge lamp. Referring to Figure 1a, the arc tube 100 is formed from light transmissive material such as quartz. The arc tube 100 defines a chamber 110 formed by pinch sealing the end portions 115, 120. An electrode assembly 122, 124 is sealed within each end portion 115, 120 to provide an electrically-conducting path from the interior of the chamber 110 to the exterior of the chamber through each end portion 115, 120. Each electrode assembly 122, 124 for a high intensity discharge arc tube 100 typically includes a discharge electrode 125, 130, electrode leads 140, 135, metallic foils 145, 150, and outer leads 155, 160. The electrode leads 135, 140 and the outer leads 155, 160 are typically connected to the metallic foils 145, 150 by spot welds.

Figure 1b is an illustration of the cross-section of a typical metallic foil 145, 150 in an electrical lead assembly 122, 124. As shown in Figure 1b, the typical foil 145, 150 is shaped in cross-section so that the thickness of the foil is greatest at the lateral center thereof, and reduces outwardly to each of the longitudinal edges. This shape has been found to reduce residual strain in the vitreous material that has been compressed around the foil during the high temperature pinching process and subsequently cooled. In a typical electrical lead assembly for an electric lamp, the foil may have a width of about 2 to 5.5 mm with a centerline thickness of about 20 to 50 µm and an edge thickness of about 3 to 7 µm. For example, a foil having a width of about 2.5 mm would typically have a centerline thickness of about 24-25 µm and an edge thickness of about 3 µm.

The assemblies 122, 124 are positioned in the end portions 115, 120 so that the foils 145, 150 are pinched between the compressed portions of the end portions 115, 120 forming the hermetic pinch seals. The assemblies 122, 124 provide the electrically conducting paths through the each end portion 145, 150 with the relatively thin foils 145, 150 providing a current path through the hermetically sealed pinch regions.

The electrode lead assemblies provide a point of failure in such lamps due to corrosion, e.g., oxidation, of the metallic foils when exposed to corrosive agents such as oxygen at high temperatures. This is primarily a problem for lamps that are operated in air, without an outer jacket, such as high wattage metal halide "sports" lamps, ultraviolet exposure lamps, HID projection light sources, and numerous incandescent tungsten halogen light sources. For example, the assemblies 122, 124 are particularly susceptible to oxidation at the outer portion of the foil 145, 150 adjacent the outer lead 155, 160 due to the exposure of this portion of the foil to oxygen or other corrosive agents during operation of the lamp. The oxidation may progress inward placing a significant amount of stress on the pinch seal. The stress may be evident from Newton rings or passageways which appear at the point at which the leads are welded to the molybdenum foil. Eventually, the electrical path may be breached or the pinch seal may crack causing the lamp to fail.

One reason for this failure is that during the formation of a pinch seal or vacuum seal with a vitreous material such as quartz, the quartz does not completely seal to the relatively thicker outer and inner lead wires, due at least in part to the relatively high viscosity of the quartz. Microscopic passageways may also be formed along the outer leads 155, 160 and also along the outer edge of the foliated portion perpendicular to the transverse axis of the lamp due to the substantial difference in the coefficient of thermal expansion of the quartz compared to that of the refractory metal outer lead wire, which is typically tungsten or molybdenum.

Another reason for this failure may also be the result of two mechanisms. First, as the molybdenum foil, wire or weld junction oxidizes, its resistance increases, leading to a further ohmic heating and higher temperatures and higher oxidation rates, eventually "burning" through the molybdenum material. Second, as the molybdenum foil, wire or weld junction oxidizes, molybdenum oxide products form. These oxides are generally less dense than the molybdenum metal materials, and the resulting expansion forces the quartz-to-metal or glass-to-metal seal apart, causing cracks and breaks. This second mechanism may also expose additional areas of molybdenum materials to air oxidation. Another common problem in pinch and shrink seals is the phenomenon referred to as "shaling." In shaling, uneven stresses in the pinch or shrink area may be caused by the adherence of the quartz to the molybdenum metal surfaces thereby resulting in minute cracks. These cracks severely weaken the glass and may lead to failure of the respective lamp from very moderate strains.

Efforts have been made in the past to prevent the oxidation of molybdenum foils in electrical assemblies that may be exposed to oxygen at high temperatures. For example, it has been proposed to reduce oxidation by coating the molybdenum foil with oxidation-protective materials such as phosphides (U.S. Pat. No. 5,387,840), aluminides, lead oxide, silicon nitride, alkali metal silicate and chromium (U.S. Pat. No. 3,793,615). Another conventional practice for protecting the molybdenum foil involves filling the open end of the pinch or shrink area with a low-melting antimony borate glass. Yet another conventional practice includes protecting the outer lead with a platinum cladding. Pinch seal assemblies comprising metal foils coated with powders of refractory metals are disclosed e.g. by US3693241 and GB671178. The utility of the aforementioned prior art approaches are marginally adequate and/or expensive; however, none of these prior art approaches includes the application of glassy films. A need, therefore, remains for oxidation-protected metallic foils for use in electrical lead assemblies for providing electrically-conducting paths through pinch seals in vitreous material and that can be exposed to high operating temperatures. It is therefore an object of the present subject matter to provide electrical lead assemblies that obviate the deficiencies of the prior art.

The present invention provides a device according to the subject-matter of claim 1 and a method according to the subject-matter of claim 7.

It will be noted that although the present invention is illustrated with these and other objectives, that the principles of the invention are not limited thereto and will include all applications of the principles set forth herein. These and other objects can be realized by simultaneous reference with the following non-exhaustive illustrative embodiments in which like segments are numbered similarly.

### BRIEF DESCRIPTION OF THE DRAWINGS

Figure 1a is a schematic representation of a conventional arc tube for a high intensity discharge lamp.

Figure 1b is an illustration of a prior art metallic foil in cross-section.

Figure 2 is a schematic representation of an arc tube.

Figure 3 is a schematic representation of a formed body arc lamp for a high intensity discharge lamp.

Figure 4 is a schematic representation of another formed-body high intensity discharge lamp.

Figure 5 is a schematic representation of a high intensity discharge lamp showing a mechanical support of arc tube and wrapped/crimped electrical connections to foil.

Figure 6 is a representation of subject matter.

### DETAILED DESCRIPTION OF THE DRAWINGS

In one embodiment of the present subject matter, a metallic foil may be coated to inhibit corrosion and the method for applying such coating. Such a foil is particularly advantageous in electrical lead assemblies because the foil may form the outer lead in the assembly and may extend beyond the end portion of the arc tube, thus eliminating the relatively thicker wire outer lead.

Also a method is provided for protecting metallic foils in electrical lead assemblies from corrosion is provided by coating the foil with a silica film, refractory abhesive and/or combination thereof. The coating provides a barrier for the foil to oxygen and other corrosive agents at high temperatures, thus reducing the corrosion of the foil and eliminating a significant cause of premature failure in electric lamps.

Another method is provided for coating metallic foil by immersing at least a portion of the foil in a bath of colloidal silica and/or silica-abhesive slurry, withdrawing the foil from the bath at a controlled rate so that silica colloid adheres to the foil, and exposing the silica colloid to a temperature sufficient to effect fusion of silica particles thereby forming a thin film of silica on the foil. Several factors may be considered in determining the thickness of the film including the viscosity of the bath, the surface tension of the bath, the temperature of the bath, and the wetting properties of the bath. The speed by which the foil is withdrawn from the bath may also be controlled. Several exemplary methods are described in parent and co-pending U.S. Patent Application No. 11/545,469 which is a divisional application of U.S. Patent No. 7,153,179; however, other methods of applying the coating to the foil may be used. For example, the coating may be applied by electrostatic spray coating, dipping, rolling, brushing and misting. Another techniques for applying the coating may include adding fine silica powder to the plume of an argon plasma torch thereby producing a spray of liquid silica.

When silica coated structures are sealed into fused vitreous material such as quartz, the coatings adhere to the vitreous material since they are the same material. Upon cooling and thermal contraction, the protective coating may peel or strip off the metal and severe shaling of the glass may be observed. Through an application of a refractory abhesive to the silica coated structures, the fused vitreous material does not adhere, and the integrity of the protective coat may be maintained. Exemplary refractory abhesive materials may be, but are not limited to, boron nitride, graphite, powders or flakes of refractory metals (such as Tungsten, Tantalum, Hafnium, Niobium, Rhenium, Osmium, etc.), or powders or flakes of refractory oxides (such as Yttrium Oxide, Zirconium Oxide, Thorium Oxide, Magnesium Oxide, Beryllium Oxide, etc.). The application of refractory abhesive materials to embodiments of the present subject matter may also prevent shaling of the silica glass caused by adherence to metal parts during pinching. Therefore, in jet-ups with or without an underlying silica coat, refractory abhesives may improve the life of a pinch or shrink seal and hence the respective arc tube or lamp by preventing the weakening of the vitreous material and by reducing the oxidation of the metal (*e.g*., slowing the access of air to the vulnerable metal). The permeability to air may be further decreased by fusible additives in the refractory abhesive formulation that promotes bonding of the refractory abhesive particles to each other and to the metal.

According to the present invention, additional protection of the foils and outer lead wires in electrical lead assemblies of electric lamps may also be achieved by mixing colloidal silica with a refractory abhesive slurry. This mixture may be applied to the assemblies by dipping, spraying, or any other suitable method. When the assembly is pinched or shrunk, the silica fuses, covering the metal with liquid silica and trapping the refractory abhesive particles in a silica matrix. Upon cooling of the assembly, the silica may remain bonded to the metal and any thermally induced cracking may occur within the silica-abhesive layer.

Certain combinations of silica-abhesive (*e.g*., silica-boron nitride, etc.) may react chemically with the metal to produce coatings of materials having exceptional oxidation protective properties. By way of a non-limiting example, it has been observed that certain mixtures of silica-boron nitride causes a melting of the molybdenum surface and creates a layer of a substance highly resistant to oxidation. In this example, the layer appears to be a molybdenum boride. Of course, other compositions of silica-abhesives may be equally effective, and such an example should not limit the scope of the claims appended herewith.

Figure 2 is a schematic representation of a pinched tube. With reference to Figure 2, outer leads in the assemblies are eliminated by extending the length of the foil. By extending the foils 113, 150, 155, the outer leads may be eliminated from the assembly. This set-up has the additional advantage of eliminating the need to adhere (spot weld, mechanical attachment, etc.) the outer leads to the foil. This will enhance the life of the lamp by avoiding the capillary formation or other such voids in the pinch seal. Further enhancement of the life of the lamp may be provided by coating any portion(s) of the foils 113, 150, 155 with an exemplary refractory abhesive or a silica-abhesive coating described above.

With reference to Figure 3, an arc tube 300 may include the chamber 110 and the end portions 115, 120 that are sealed by pinching. The lead assemblies may include electrode leads 135, 140, foils 145, 150, and outer leads 155, 160. Enhancement of the life of the arc tube 300 may be provided by coating any portion(s) of the end portions 115, 120 and/or the lead assemblies including the electrode leads 135, 140, foils 145, 150 and outer leads 155, 160 with an exemplary refractory abhesive or a silica-abhesive coating described above.

With reference to Figure 4, each of foils 150, 155 may be extended beyond the respective end portions 115, 120 of the arc tube 400 thereby eliminating the outer leads from the assemblies. Of course, enhancement of the life of the arc tube 400 may be provided by coating any portion(s) of the end portions 115, 120 and/or foils 150, 155 with an exemplary refractory abhesive or a silica-abhesive coating described above.

Figure 5 is a schematic representation of a high intensity discharge lamp showing a mechanical support for arc tube and wrapped/crimped electrical connections to the foil. High intensity discharge lamp 500 includes an arc tube 505 supported with the outer lamp envelope 508 of the lamp 500. The arc tube 505 includes a bulbous chamber 510 intermediate tubular end portions 512, 514. The arc tube 505 is mechanically secured within the envelope by supporting the arc tube at the end portions 512, 514 thereof. The electrical assemblies of the arc tube include metallic foils 515, 525 that extend beyond the end portions 512, 514 to provide electrical connections for the arc tube. The electrical leads connecting the lamp base to the foils are mechanically and electrically secured to the foils by coil connections 527, 528. Although the foils 515, 525 are not as mechanically rigid as the outer leads in conventional lead assemblies, mechanical deformation of the foils is minimized by supporting the arc tube 505 from the end portions 512, 514. Enhancement of the life of the arc tube 500 may be provided by coating any portion(s) of the electrical assemblies of the arc tube 500 including the foils 515, 525 with an exemplary refractory abhesive or a silica-abhesive coating described above.

With reference to Figure 6, a method 600 of providing an electrical connection through a pinch or shrink seal formed in a quartz or glass body is illustrated. At step 610, a quartz or glass body having at least one open end is provided, and at step 620, an electrical lead assembly comprising a metallic foil is also provided.
The metallic foil may be formed from molybdenum, however, such an example should not limit the scope of the claims appended herewith as the metallic foil may be formed from any suitable metal or material. At step 630, a coating comprising a refractory abhesive may be applied to at least a portion of the metallic foil. The refractory abhesive may be, but is not limited to, boron nitride, graphite, powders or flakes of refractory metals, and powders or flakes of refractory oxides. The application of the refractory abhesive may include mixing colloidal silica with a refractory abhesive slurry and applying the mixture to at least a portion of the metallic foil. The electrical lead assembly may be positioned in an open end of the body at step 640, and the open end of the body may be pinch or shrink sealed so that the quartz or glass of the body forms a hermetic seal around the metallic foil of the electrical lead assembly at step 650.

### Example 1

Several electrode assemblies commonly utilized in 2000 Watt arc tubes were coated by dipping the assemblies into a bath containing an aqueous silica colloidal mixture. The mixture included:

| | |
|---|---|
| ST-OUP (from Nissan Chemical Corp.) | 9.0 gm |
| Water | 7.0 gm |
| Concentrated ammonia | 1.0 gm |
| Polyvinylpyrrolidone, 1% aqueous solution | 6.0 gm |
| NaBO₂, 5% aqueous solution | 1.6 gm |

After drying, the assemblies were overcoated with an exemplary refractory abhesive, specifically, (1) graphite (TC-2 from Fiber Materials, Inc.) diluted 1:1 with amyl acetate, and (2) boron nitride (BN Aerosol Brushable, Zyp Coatings). These exemplary assemblies were pinched into quartz lamp arc tubes, and then freed from the glass with a diamond saw. When anodically oxidized in 4% HCl, little blackening was observed, thereby illustrating that the "green" coat fused to the molybdenum parts. Both boron nitride and graphite coatings exhibited excellent oxidation properties.

### Example 2

Several electrode assemblies commonly utilized in 2000 Watt arc tubes were coated by dipping the assemblies into a bath containing an aqueous silica colloidal mixture. The mixture included:

| | |
|---|---|
| ST-OUP (from Nissan Chemical Co.) | 9.0 gm |
| Water | 7.0 gm |
| Concentrated ammonia | 1.0 gm |
| Polyvinylpyrrolidone, 1% aqueous solution | 6.0 gm |
| NaBO₂, 5% aqueous solution | 1.6 gm |

After drying, the assemblies were overcoated with an exemplary refractory abhesive only up to the outer lead weld. The refractory abhesives were (1) graphite (TC-2 from Fiber Materials, Inc.) diluted 1:1 with amyl acetate, and (2) boron nitride (BN Aerosol Brushable, Zyp Coatings). Several exemplary assemblies were placed in an oven at 400°C and several were assembled into lamps. Testing indicated a significant reduction in oxidation rates of the coated foil/lead assemblies when compared to uncoated assemblies, with significant increases in lamp life.

### Example 3

Pieces of molybdenum foil and/or lead junctions and weld spots of bare assemblies, having no silica coatings were provided with a refractory abhesive coating, namely, boron nitride. Boron nitride coatings were also applied to the electrode shank/foil junctions. The refractory abhesive coatings provided no negative impact on the internal lamp operating characteristics. In comparison, lamps made with bare foil/lead assemblies illustrated a typical failure within 500 hours of operation; however, lamps made with the exemplary refractory abhesive coating of boron nitride exhibited no oxidation damage at 500 hours of operation.

### Example 4

Pieces of molybdenum foil and/or lead junctions and weld spots of bare assemblies, having no silica coatings were provided with a refractory abhesive coating, namely, a mixture of silica and boron nitride. Exemplary lamps made with this refractory abhesive coating exhibited excellent oxidation protection at 400°C for several thousand hours of operation.

It is to be understood that the set-ups described are illustrative only and the scope of the invention is to be defined solely by the appended claims.

## Claims

1. A device comprising:
a quartz or glass body forming a chamber and having one or more pinch or shrink seals formed in the body; and
an electrical lead assembly suitable for providing an electrical connection through a pinch seal in a quartz or glass body, said assembly comprising a metallic foil having a coating on at least a portion thereof comprising a refractory abhesive; wherein the refractory abhesive is a material having the capability of resisting adhesion to the quartz or glass body and is selected from the group consisting of boron nitride, graphite, powders or flakes of refractory metals, and powders or flakes of refractory oxides;
wherein the metallic foil is positioned within the pinch or shrink seal, and **characterized in that** said coating also comprises colloidal silica.

2. The device of Claim 1 wherein said metallic foil is formed from molybdenum.

3. The device of claim 1 or 2 wherein said refractory abhesive comprises boron nitride.

4. The device of one of the preceding claims comprising a film on at least a portion of said foil, said film comprising a compound containing metal from said foil.

5. The device of claim 4 wherein the metallic foil is formed from molybdenum and said film comprises a compound of molybdenum.

6. The device of Claim 5 wherein said compound of molybdenum is formed by chemical reaction between one or more elements in said coating and said foil.

7. A method of providing an electrical connection through a pinch or shrink seal formed in a quartz or glass body, said method comprising:
providing a quartz or glass body having at least one open end;
providing an electrical lead assembly comprising a metallic foil;
applying a coating comprising a colloidal silica and a refractive abhesive to at least a portion of the metallic foil, wherein the refractory abhesive is a material having the capability of resisting adhesion to the quartz or glass body and is selected from the group consisting of boron nitride, graphite, powders or flakes of refractory metals and powders or flakes of refractory oxides;
positioning the electrical lead assembly in an open end of the body;
pinch or shrink sealing the open end of the body so that the quartz or glass of the body forms a hermetic seal around the metallic foil of the electrical lead assembly.

8. The method of Claim 7 wherein the metallic foil is formed from molybdenum.

9. The method of claims 7 or 8 wherein the step of applying a coating comprising a refractory abhesive to at least a portion of the metallic foil comprises mixing said colloidal silica with a refractory abhesive slurry and applying the mixture to at least a portion of the metallic foil.

10. The method of one of claims 7 to 9, wherein the step of applying a coating comprises:
applying a protective layer comprising fusible glass precursors to at least a portion of the electrical lead assembly;
applying a layer of material over at least a portion of the protective layer, the material being suitable for preventing adhesion of the protective layer overlaid by the material and the glass body when the electrical lead assembly is sealed within a pinch or shrink seal in the body.

11. The method of one of claims 7 to 9, wherein the step of applying a coating comprises:
applying a protective layer to at least a portion of the electrical lead assembly, the protective layer comprising fusible glass precursors and a material which prevents mechanically strong bonding of the protective layer to the glass body when the electrical lead assembly is sealed within a pinch or shrink seal in the body.

## Patentansprüche

1. Vorrichtung, die Folgendes umfasst:
Einen Quarz- oder Glaskörper, der eine Kammer bildet und der eine oder mehrere Quetsch- oder Schrumpfdichtungen umfasst, die in dem Körper gebildet sind; und
eine elektrische Leiteranordnung, die geeignet ist, eine elektrische Verbindung bereitzustellen, die sich durch eine Quetschdichtung in dem Quarz- oder Glaskörper erstreckt, wobei die Anordnung eine metallische Folie umfasst, die zumindest abschnittsweise eine Beschichtung aufweist, die ein hitzebeständiges abhäsives Material umfasst; wobei das hitzebeständige abhäsive Material die Eigenschaft hat, sich einem Anhaften an den Quarz- oder Glaskörper zu widersetzen, und wobei das abhäsive Material aus einer Gruppe gewählt ist, die aus Folgendem besteht: Bornitrid, Graphit, Pulver oder Flocken hitzebeständiger Metalle und Pulver oder Flocken hitzebeständiger Oxide; wobei die metallische Folie innerhalb der Quetsch- oder Schrumpfdichtung angeordnet ist, und
**dadurch gekennzeichnet, dass** die genannte Beschichtung weiterhin kolloidales Siliziumoxid umfasst.

2. Vorrichtung nach Anspruch 1, bei der die metallische Folie aus Molybdän gebildet ist.

3. Vorrichtung nach Anspruch 1 oder 2, bei der das hitzebeständige abhäsive Material Bornitrid enthält.

4. Vorrichtung nach einem der vorgenannten Ansprüche, die auf zumindest einen Teil der Folie einen Film aufweist, wobei der Film einen Verbund umfasst, der Metall der Folie enthält.

5. Vorrichtung nach Anspruch 4, bei welcher die metallische Folie aus Molybdän gebildet ist und der Film einen Molybdänverbund enthält.

6. Vorrichtung nach Anspruch 5, bei welcher der Molybdänverbund durch eine chemische Reaktion zwischen einem oder mehreren Elementen in der Beschichtung und der Folie gebildet ist.

7. Verfahren zum Bereitstellen einer elektrischen Verbindung durch eine Quetsch- oder Schrumpfdichtung hindurch, die in einem Quarz- oder Glaskörper gebildet ist, wobei das Verfahren die folgenden Schritte umfasst:
Bereitstellen eines Quarz- oder Glaskörpers, der zumindest ein offenes Ende umfasst;
Bereitstellen einer elektrischen Leiteranordnung, die eine metallische Folie umfasst;
Aufbringen einer Beschichtung auf zumindest einen Teil der metallischen Folie, wobei die Beschichtung kolloidales Siliziumoxid und ein hitzebeständiges abhäsives Material umfasst, wobei das hitzebeständige abhäsive Material die Eigenschaft hat, sich einem Anhaften an den Quarz- oder Glaskörper zu widersetzen, und wobei das hitzebeständige abhäsive Material aus einer Gruppe gewählt ist, die Folgendes umfasst: Bornitrid, Graphit, Pulver oder Flocken hitzebeständiger Metalle und Pulver oder Flocken hitzebeständiger Oxide;
Anordnen der elektrischen Leiteranordnung in einem offenen Ende des Quarz- oder Glaskörpers;
Abdichten des offenen Endes des Quarz- oder Glaskörpers durch Quetschen oder Schrumpfen, so dass das Quarz oder das Glas des Körpers eine hermetische Dichtung um die metallische Folie der elektrischen Leiteranordnung bildet.

8. Verfahren nach Anspruch 7, bei dem die metallische Folie aus Molybdän gebildet ist.

9. Verfahren nach Anspruch 7 oder 8, bei dem der Schritt des Aufbringens einer Beschichtung, die zumindest einen Teil der hitzebeständiges abhäsives Material umfasst, auf die zumindest einen Teil der metallischen Folie die folgenden Schritte umfasst:
Mischen des kolloidalen Siliziumoxids mit einem Brei des hitzebeständigen abhäsiven Materials und
Aufbringen der Mischung auf zumindest einen Teil der metallischen Folie.

10. Verfahren nach einem der Ansprüche 7 bis 9, bei dem der Schritt des Aufbringens einer Beschichtung die folgenden Schritte umfasst:
Aufbringen einer Schutzschicht, die eine schmelzbare Glasvorstufe umfasst, auf zumindest einen Teil der elektrischen Leiteranordnung;
Aufbringen eines Materials auf zumindest einen Teil der Schutzschicht, wobei das Material geeignet ist, ein Anhaften der mit dem Material überzogenen Schutzschicht an dem Glaskörper zu verhindern, wenn die elektrische Leiteranordnung innerhalb einer Quetsch- oder Schrumpfdichtung des Körpers dicht eingeschlossen wird.

11. Verfahren nach einem der Ansprüche 7 bis 9, bei dem der Schritt des Aufbringens der Beschichtung den folgenden Schritt umfasst:
Aufbringen einer Schutzschicht auf zumindest einen Teil der elektrischen Leiteranordnung, wobei die Schutzschicht eine schmelzbare Glasvorstufe und ein Material umfasst, wobei das Material verhindert, dass die Schutzschicht und der Glaskörper eine starke mechanische Verbindung eingehen, wenn die elektrische Leiteranordnung innerhalb einer Quetsch- oder Schrumpfdichtung des Körpers dicht eingeschlossen wird.

## Revendications

1. Dispositif comprenant:
un corps en quartz ou en verre formant une chambre et possédant un ou plusieurs joints à pincement ou rétractables formés dans le corps ; et
un assemblage de fils électriques adapté pour fournir une connexion électrique par le biais d'un joint à pincement dans un corps en quartz ou en verre, ledit assemblage comprenant une feuille métallique possédant un revêtement sur au moins une partie de celle-ci comprenant un agent anti-adhérent réfractaire ; dans lequel l'agent anti-adhérent réfractaire est un matériau ayant la capacité de résister à l'adhérence au corps en quartz ou en verre et est choisi dans le groupe constitué du nitrure de bore, du graphite, des poudres ou des paillettes de métaux réfractaires, et des poudres ou des paillettes d'oxydes réfractaires ;
dans lequel la feuille métallique est positionnée à l'intérieur du joint à pincement ou rétractable, et **caractérisé en ce que** ledit revêtement comprend également de la silice colloïdale.

2. Dispositif selon la revendication 1 dans lequel ladite feuille métallique est fabriquée à partir de molybdène.

3. Dispositif selon la revendication 1 ou 2 dans lequel ledit agent anti-adhérent réfractaire comprend du nitrure de bore.

4. Dispositif selon l'une quelconque des revendications précédentes comprenant un film sur au moins une partie de ladite feuille, ledit film comprenant un composé contenant un métal de ladite feuille.

5. Dispositif selon la revendication 4 dans lequel la feuille métallique est fabriquée à partir de molybdène et ledit film comprend un composé de molybdène.

6. Dispositif selon la revendication 5 dans lequel ledit composé de molybdène est fabriqué par réaction chimique entre un ou plusieurs éléments dudit revêtement et de ladite feuille.

7. Procédé servant à créer une connexion électrique par le biais d'un joint à pincement ou rétractable formé dans un corps en quartz ou en verre, ledit procédé comprenant :
la fourniture d'un corps en quartz ou en verre possédant au moins une extrémité ouverte ;
la fourniture d'un assemblage de fils électriques comprenant une feuille métallique ;
l'application d'un revêtement comprenant une silice colloïdale et un agent anti-adhérent réfractaire sur au moins une partie de la feuille métallique, dans lequel l'agent anti-adhérent réfractaire est un matériau ayant la capacité de résister à l'adhérence au corps en quartz ou en verre et est choisi dans le groupe constitué du nitrure de bore, du graphite, des poudres ou des paillettes de métaux réfractaires et des poudres ou des paillettes d'oxydes réfractaires ;
le positionnement de l'assemblage de fils électriques dans une extrémité ouverte du corps ;
la fermeture par pincement ou rétraction de l'extrémité ouverte du corps de manière à ce que le quartz ou le verre du corps forme un joint hermétique autour de la feuille métallique de l'assemblage de fils électriques.

8. Procédé selon la revendication 7 dans lequel la feuille métallique est fabriquée à partir de molybdène.

9. Procédé selon les revendications 7 ou 8 dans lequel l'étape consistant à appliquer un revêtement comprenant un agent anti-adhérent réfractaire sur au moins une partie de la feuille métallique comprend le mélange de ladite silice colloïdale avec une suspension concentrée d'agent anti-adhérent réfractaire et l'application du mélange sur au moins une partie de la feuille métallique.

10. Procédé selon l'une des revendications 7 à 9, dans lequel l'étape consistant à appliquer un revêtement comprend :
l'application d'une couche de protection comprenant des précurseurs de verre fusibles sur au moins une partie de l'assemblage de fils électriques ;
l'application d'une couche de matériau sur au moins une partie de la couche de protection, le matériau étant adapté pour prévenir l'adhérence de la couche de protection recouverte par le matériau et le corps en verre lorsque l'assemblage de fils électriques est enfermé hermétiquement à l'intérieur d'un joint à pincement ou rétractable dans le corps.

11. Procédé selon l'une des revendications 7 à 9, dans lequel l'étape consistant à appliquer un revêtement comprend : l'application d'une couche de protection sur au moins une partie de l'assemblage de fils électriques, la couche de protection comprenant des précurseurs de verre fusibles et un matériau qui prévient mécaniquement la forte adhérence de la couche de protection au corps en verre lorsque l'assemblage de fils électriques est enfermé hermétiquement à l'intérieur d'un joint à pincement ou rétractable dans le corps.
